

# UNITED STATES PATENT OFFICE.

JAMES F. O'BRIEN, OF CHICAGO, ILLINOIS.

## EXPLOSIVE.

1,070,837.

Specification of Letters Patent. Patented Aug. 19, 1913.

No Drawing.

Application filed June 3, 1912. Serial No. 701,258.

*To all whom it may concern:*

Be it known that I, JAMES F. O'BRIEN, a citizen of the United States, residing at Chicago, in the county of Cook, State of Illinois, have invented new and useful Improvements in Explosives, of which the following is a specification.

This invention relates to variations and improvements in my explosives of the chlorate carbo-hydrate class for which I have filed various applications for United States Letters Patent important among which are my applications entitled Explosives, filed Sept. 5, 1911, bearing S. N. 647,474, filed 10 Sept. 20, 1911, bearing S. N. 650,373; filed 15 Oct. 2, 1911, bearing S. N. 652,390; filed Oct. 21, 1911, bearing S. N. 656,529; filed January 11, 1912, bearing S. N. 670,645; filed Feb. 19, 1912, bearing S. N. 678,708. 20 In these applications I have described and claimed in general an explosive consisting of a chlorate of an alkali metal, a carbo-hydrate and a silico-aluminous material. In my co-pending application entitled Explosives, filed June 3rd 1912 bearing S. N. 25 701,257 I have set forth the application of silica (silicon dioxide) to my formerly described explosives. And in this present application I wish to set forth the use of a carbonaceous or hydro-carbonaceous material in combination with a chlorate and a carbo-hydrate and the silicious material.

I use a preferably liquid carbonaceous or hydro-carbonaceous material in combination 30 with the chlorate, carbo-hydrate and silicious material, primarily for producing a plastic packable explosive which may be formed into a cartridge or stick after the manner of dynamite.

40 The carbonaceous or hydro-carbonaceous material may be one of many different substances. In practice I may employ crude petroleum, or a divisional product thereof, using a small amount of free carbon or coal dust with the liquid.

The following formula broadly shows the composition of my explosive:

|                       |          |
|-----------------------|----------|
| Chlorate              | 30 parts |
| Carbo-hydrate         | 10 "     |
| Carbonaceous material | 5 "      |
| Silicious material    | 55 "     |

50 or the silicious material may be more or less than the above given proportions. I generally maintain the three to one proportion 55 of the chlorate and carbo-hydrate; and the

carbonaceous material generally is about five per cent. of the total weight of explosive. But the amount of silicious material may vary, depending upon the character and quality of powder desired.

60 A preferred formula is as follows:

|                    |          |
|--------------------|----------|
| Potassium chlorate | 30 parts |
| Starch             | 10 "     |
| Coal dust          | 1 "      |
| Crude petroleum    | 4 "      |
| Silicious material | 55 "     |

70 This formula in practice may be carried out as follows: The chlorate and starch (either in the form of pure starch or in the form of starch carried by cereal flour) are thoroughly mixed after having been pulverized or otherwise broken into small parts. The silicious material (say in the form of 75 silica) and the chlorate and starch are thoroughly mixed together, and during this mixing operation the liquid carbonaceous material (crude oil) is slowly introduced and distributed over the dry materials and 80 thoroughly mixed therewith. The resultant mass is just sufficiently plastic to form a cohesive body and to be easily packed into cartridges to form sticks. The coal dust is supplied during the mixing operation and 85 is useful largely for propagating the flame of explosions through the mass of explosive, making it necessary to use the blasting cap. The explosive as thus prepared needs no water proofing, being entirely water 90 proof in itself.

I may substitute any of the non-volatile divisional products of crude oil, a distillate being extremely advantageous in my explosive composition. When using distillate I use a small quantity of de-odorizing substances to overcome the distillate odor, amyl acetate being suitable. A few drops of this material in a large quantity of explosive will overcome the distillate odor.

95 This explosive herein described has all of the advantages before described by me in connection with my explosives above referred to. It is capable of manufacture by a cold frictionless, non-confined process; it 105 will not deteriorate on exposure; and it is extremely safe to handle. Its explosive energy is favorably comparable with that of sixty to eighty per cent. dynamite, and it has the advantage of localizing its explosive effects in the manner so much desired in blasting and similar operations. This 110

last named advantage is very important in the present described explosive as the work of blasting and the like is precisely that for which this explosive is designed. These advantages are due to my combination as set forth. The silicious material imparts to the explosive a certain explosive energy; that is a silicious matter added to a mixture of chlorate and carbo-hydrate will increase 10 the total explosive energy of the mixture. And the liquid carbonaceous substance not only mechanically effects the finished powder but it enters into the explosive reaction and contributes to the total explosive energy. These two ingredients are so cheap 15 that the complete explosive is more energetic, cost for cost, than an explosive without them.

Having described my invention, I claim:

20 1. An explosive, comprising a chlorate of an alkali metal, a carbo-hydrate, hydro-carbonaceous material and silica.

2. An explosive, comprising a chlorate of an alkali metal and a carbo-hydrate in the

approximate proportions three to one, hydro-carbonaceous material and silica.

3. An explosive, comprising potassium chlorate, a carbo-hydrate, a liquid hydro-carbon, and silica.

4. An explosive, consisting of potassium 30 chlorate, a carbo-hydrate, crude oil, coal dust, and silica.

5. An explosive, consisting of potassium chlorate 30 parts, carbo-hydrate 10 parts, silica up to approximately 55 parts, and 35 carbon and liquid hydro-carbon together 5 parts.

6. An explosive, consisting of potassium chlorate, carbo-hydrate, a liquid carbonaceous material, and silica.

In witness that I claim the foregoing I have hereunto subscribed my name this 24th day of May 1912.

JAMES F. O'BRIEN.

Witnesses:

JEROME McNABB,  
ELWOOD H. BARKELEW.

Copies of this patent may be obtained for five cents each, by addressing the "Commissioner of Patents, Washington, D. C."